

# UNITED STATES PATENT OFFICE.

JOHN COLLINS CLANCY, OF NEW YORK, N. Y.

## TREATMENT OF ORES BEARING PRECIOUS METALS.

971,252.

Specification of Letters Patent. Patented Sept. 27, 1910.

No Drawing.

Application filed March 13, 1909. Serial No. 483,331.

*To all whom it may concern:*

Be it known that I, JOHN COLLINS CLANCY, a subject of the King of Great Britain, having declared my intention of becoming a citizen of the United States, at present residing at New York city, borough of Manhattan, in the county of New York and State of New York, have invented certain new and useful Improvements in the

10 Treatment of Ores Bearing Precious Metals, of which the following is a specification.

My invention relates to a novel method of treating auriferous ores, which method is particularly described and pointed out in

15 the following specification and claim.

I have discovered that gold may be advantageously recovered from ores containing the same, whether such ores be rebellious or non-rebellious, by the use of a solution 20 containing a soluble iodid and a suitable substance capable of yielding nascent oxygen in said solution. In the case of rebellious ores—those containing, for example, reducing agents, or tellurium, or both—no 25 preliminary treatment, such as roasting, is required.

One way of carrying my invention into practice, whether reducing agents and tellurium be or be not present, is to treat the 30 pulverized ores simultaneously with a solution—such, for example, as potassium iodid—a soluble persulfate—such, for example, as the sodium of ammonium persulfate. The desired result is accomplished if

35 the solution be substantially acid, although it will take place if the solution be neutral or alkaline or only slightly acid. The strength of the solution is, to some extent, dependent upon the character of the ore to

40 be treated, and it must, therefore, be ascertained by preliminary tests; but in practice with certain ores such as we have treated, we have found the following proportions to

45 answer well the purposes of the process: a solution containing one pound potassium iodid, three pounds sodium persulfate and

one-half pound of lime or soda dissolved in two thousand pounds of water in the proportion of two parts of the above named

50 solution to one part of ore. The same solution can be used again and again by keeping up the requisite strength in potassium iodid and sodium persulfate, but no further addition of potassium iodid is necessary, except

55 to compensate for mechanical losses, as the persulfate regenerates the iodin to begin its

work over again. Between each operation it is desirable to pass the liquor through zinc shavings in the ordinary way to extract the values which it contains. 60

Another way of carrying my invention into practice, effecting the solution of the gold, whether reducing agents and tellurium be or be not present, is to treat the pulverized ore simultaneously with a soluble iodid 65 solution—such, for example, as potassium iodid—and ozone or ozonized air. In practice with certain ores I have treated, I have found the following proportions to answer well the purposes of the process: a solution of one pound of potassium iodid and one-half pound of lime or soda, dissolved in two thousand pounds of water in the proportion of two parts of said solution to one part of ore. The amount of ozone to be passed into 70 the solution is to be determined by titration, or otherwise. In practice I have found that a proportion equivalent to two hundred grams of ozone to two thousand pounds of solution gave good results, although with 75 some ores as little as fifteen grams of ozone to two thousand pounds of solution have given excellent results. In this case also the ozone regenerates the iodin to begin its work over again. Hence, no further addition of 80 potassium iodid is necessary except to compensate for mechanical losses.

It will be understood that the amount of gold carried by the gold-bearing ore is very small, and that when subjected to the potassium iodid, and ozone, will be held in solution in the form of auric iodid, and in view of the very small amount of gold present the quantity of iodin drawn from the solvent will be correspondingly small. 95

Another way of carrying my invention into practice is to substitute in the above example nitrogen oxid—such, for example, as nitrogen peroxid—for the ozone there used. Here, again, the peroxid of nitrogen 100 regenerates the iodin as in the other examples.

As I have said, it is not necessary in practicing the above processes with rebellious ores—those containing, for example, reducing agents (sulfids of iron, etc.) or tellurium, or both—to roast the ore, since the sulfids do not act on the solution to decompose it, and the tellurium is dissolved simultaneously with the precious metal. 105

When the solution is to be reused, the oxidizing agents may be added thereto, if 110

necessary, after each treatment when the solution is withdrawn from the ore, so as to place the solution in proper condition for the next subsequent treatment.

5 The cost of iodin in a commercial process would be prohibitive were it not for the fact that in the processes above described the iodin is repeatedly regenerated and does the same work over and over again. Its action 10 may be likened to that of a vehicle or carrier and hence it is not substantially consumed.

It will be understood that various modifications and changes in the described process 15 may be made without departing from the spirit of my invention and without exceeding the scope of my claim.

Having thus described my invention, what I claim and desire to secure by Letters Patent of the United States is:—

20

The method of treating pulverized ore containing gold, which consists in subjecting said ore to the action of a solution containing a soluble iodid and a substance capable of yielding nascent oxygen in the presence 25 of said solution.

In testimony whereof I have signed my name to this specification in the presence of two subscribing witnesses.

JOHN COLLINS CLANCY.

Witnesses:

W. A. PAULING,  
OSCAR ASCHER.